

## UNITED STATES PATENT OFFICE

2,095,070

## DYEING SKINS OR PELTS

Erich Lehmann, Priorau, Kreis Bitterfeld, Germany, assignor to General Aniline Works, Inc., New York, N. Y., a corporation of Delaware

No Drawing. Application January 8, 1937, Serial No. 119,587. In Germany January 24, 1936

6 Claims. (Cl. 8—5)

The present invention relates to a new process for dyeing skins and pelts.

In my copending application Serial No. 741,876 I have disclosed a process for dyeing pelts and hairs by treating these materials in a bath containing an oxidizing agent and a salt-like compound of the general formula



10 wherein R is inter alia a polyhydroxy compound of the naphthalene series and R' is an unsubstituted or substituted aminophenyl radicle, these compounds being used if necessary in the presence of a dispersing agent for the purpose of bringing substances of the said kind which are sparingly soluble in water into the desired fine state of distribution.

Now I have found that with like effect salt-like compounds may be used which correspond to 20 the general formula



wherein x is H or OH, y is halogen, nitro, aceto and halogenaceto and R means an aromatic or 30 heterocyclic base.

With the help of capillary active substances the sparingly water-soluble salts of this kind may be used as dyestuffs for pelts and there are obtained by this means beautiful and strong tints 35 of good fastness.

The following examples illustrate the invention, the parts being by weight:—

Example 1.—2 parts of the mixture consisting of 40 parts of the salt made from 4-aceto-1,2-dihydroxybenzene and 4-aminodiphenylamine and 60 parts of a dispersing agent made as described in German specification No. 436,881 by condensation of a naphthalene sulfonic acid with benzylchloride, are dissolved in 1000 parts of water and the solution is mixed with 10 parts of hydrogen peroxide of 3 per cent. strength. A white rabbit skin previously prepared with chromium salt which is dyed in this bath for 3 hours at a temperature of 30° C. acquires a green-gray tint which has good fastness to light.

Example 2.—2 parts of a mixture consisting of 40 parts of the salt made from 8-aminoquinoline and 4-chloro-1,2-dihydroxybenzene and 60 parts of the wetting agent mentioned in Example 1, are dissolved in 1000 parts of water and

the solution is mixed with 10 parts of hydrogen peroxide solution of 3 per cent. strength. A white lamb skin pre-treated with potassium bichromate is dyed in this bath for 3 hours at 30° C. whereby a clear reddish brown is obtained. 5

Example 3.—2 parts of a mixture consisting of 40 parts of the salts made from 4-nitro-1,3-dihydroxybenzene and 4-nitro-1,3-diaminobenzene and 60 parts of isopropylnaphthalene sulfonic acid are dissolved in 1000 parts of water 10 and the solution is mixed with 10 parts of a hydrogen peroxide solution of 3 per cent. strength. A white rabbit skin pre-treated with an iron mordant is dyed by this dye under conditions the same as described in Example 2 a clear green 15 yellow.

Example 4.—2 parts of a mixture consisting of 40 parts of the salt made from 5-nitro-1,2,4-trihydroxybenzene and 2,4-diaminotoluene and 60 parts of Turkey red oil are dissolved in 1000 parts of water and the solution is mixed with 10 parts of hydrogen peroxide solution of 2 per cent. strength. A white lamb skin pre-treated with a chromium mordant is dyed green-brown by this 20 bath. 25

Example 5.—2 parts of a mixture consisting of 40 parts of the salt from 1,5-diaminonaphthalene and 4-trichloraceto-1,2-dihydroxybenzene and 60 parts of isopropylnaphthalene sulfonic acid are dissolved in water and the solution is mixed with 10 parts of a hydrogen peroxide solution of 3 per cent. strength. A white rabbit skin pre-treated with a chromium mordant is dyed a 30 full bluish gray tint in this bath. 35

Example 6.—2 parts of a mixture consisting of 40 parts of the salt made from 4-bromo-1,2,6-trihydroxybenzene and 2-chloro-1,4-diaminobenzene and 60 parts of Turkey red oil are dissolved in 1000 parts of water and the solution is mixed with 10 parts of a hydrogen peroxide solution of 3 per cent. strength. A white lamb skin previously treated with an iron mordant is dyed a 40 green-gray tint in this bath. 45

The salt-like addition products used as pelt dyes according to my invention, are readily prepared in the manner described in "Organische Molekulverbindungen" by Paul Pfeiffer, 2nd Edition, page 270-271, or Liebig's Annalen, vol. 438, page 74 et seq., by dissolving the amine and the hydroxy compound in equimolecular proportions 50 in an appropriate solvent, mixing the solutions and, if necessary, eliminating the solvent.

It is obvious that my invention is not limited to the foregoing examples or to the specific details given therein. Other dispersing agents such 55

as, for instance, sulfonated hydrocarbons from brown coal tar, sulfonated solar oil, water-soluble condensation products of unsaturated fatty acids with sulfonic acids of aromatic compounds, aliphatic alcohol sulfonates or the like, may be used for dissolving or dispersing the salt-like products in question. In the examples I have given a number of these salt-like compounds of substituted polyhydroxybenzenes and amines. These may be substituted, however, by similar compounds containing other basic components and generally this basic substituent may be a 1,3- or 1,4-diaminobenzene unsubstituted or substituted in the nucleus or in one of the NH<sub>2</sub> groups, furthermore, it may be 1,4-, 1,5-, 2,4-, 2,7-diaminonaphthalene, benzidine and their derivatives. From the heterocyclic series I enumerate 8-aminoquinoline, 8-aminoquinaldine, 5,8-diaminoquinoline and 3-aminocarbazole.

20 What I claim is:—

1. The process for dyeing skins and pelts which comprises treating the said materials in a bath containing an oxidizing agent, a dispersing agent and a salt-like compound of the general formula



wherein *x* is a member of the group consisting of H and OH, *y* is a member of the group consisting of halogen, nitro, aceto and halogenoaceto, and *R* means the radicle of a base of the group consisting of aminobenzenes, aminonaphthalenes and heterocyclic bases.

2. The process for dyeing skins and pelts which comprises treating the said materials in a bath containing an oxidizing agent, a dispersing agent and a salt-like compound of the general formula



50 wherein *y* is a member of the group consisting of halogen, nitro, aceto and halogenoaceto and *R* means the radicle of a base of the group consisting of aminobenzenes, aminonaphthalenes and heterocyclic bases.

3. The process for dyeing skins and pelts which comprises treating the said materials in a bath containing an oxidizing agent, a dispersing agent and a salt-like compound of the general formula



wherein *y* is a member of the group consisting of halogen, nitro, aceto and halogenoaceto and *R* means the radicle of a base of the group consisting of aminobenzenes, aminonaphthalenes and heterocyclic bases.

4. The process for dyeing skins and pelts which comprises treating the said materials in a bath containing an oxidizing agent, a dispersing agent and a salt-like compound of the formula



5. The process for dyeing skins and pelts which comprises treating the said materials in a bath containing an oxidizing agent, a dispersing agent and a salt-like compound of the formula



6. The process for dyeing skins and pelts which comprises treating the said materials in a bath containing an oxidizing agent, a dispersing agent and a salt-like compound of the formula



ERICH LEHMANN.